

Dec. 23, 1958

**J. ZOLDAS**  
APPARATUS FOR PRODUCING SHEET  
METAL BY ELECTRODEPOSITION  
Filed May 14, 1956

**2,865,830**



FIG. 2



FIG. 3



## INVENTOR

John Zoldas

BY JOHN ZOLDAK  
Pamela Edwards, Walter Barnes & Taylor

## ATTORNEYS

1

2,865,830

## APPARATUS FOR PRODUCING SHEET METAL BY ELECTRODEPOSITION

John Zoldas, Perth Amboy, N. J., assignor to The Anaconda Company, New York, N. Y., a corporation of Montana

Application May 14, 1956, Serial No. 584,716

5 Claims. (Cl. 204—208)

This invention relates to producing sheet metal by electrodeposition on a rotating drum cathode, and then stripping the electrodeposit from the drum. The invention is particularly directed to the provision of an improved method of carrying out the electrodeposition operation so as to produce an electrodeposited sheet of improved surface quality and of improved uniformity of gage across the width of the cathode drum on which it is formed. The invention also provides improvements in the apparatus used for producing electrodeposited sheet metal in accordance with the new method.

Numerous proposals have been made heretofore for producing a variety of metals in sheet form by electrodeposition on a rotating drum cathode, and sheet copper has been thus produced on a commercial scale for many years. The electrodeposition method has the advantage that sheets of wide width, thin gage, and indefinitely long lengths can be produced. Sheet metal made in this manner, however, is subject to considerable variation in thickness across the width of the sheet; and it is difficult to produce metal of very thin gage (weighing, say, one ounce or less per square foot, in the case of copper) that is free from pinholes. Heretofore the only way by which it has been possible to produce electrodeposited sheet copper having sufficient uniformity of gage and freedom from pinholes, in thicknesses corresponding to weights of one ounce to two ounces per square foot, has been to subject the electrolyte between the cathode drum and the nearby anode to intense air agitation.

While air agitation has been necessary to produce electrodeposited sheet copper of acceptable quality, such agitation is by no means free from objection. It causes much splashing of the electrolyte, with the result that the atmosphere in the vicinity of the electrodeposition equipment becomes charged with an irritating acid mist. Workmen in the area must wear some form of respiratory protective apparatus, and the acid mist promotes discoloration and even damaging corrosion to the electrodeposited sheet. Splashing and sloshing of the electrolyte near the cathode drum also results in wetting and trapping of specks of lead dust (generated by the cathode polishing apparatus) on the surface of the cathode drum, leading to a defect in the deposited sheet metal known as "leaded porosity." And of course the splashing of electrolyte and the acid mist in the vicinity of the electrodeposition equipment promotes rapid corrosion of the apparatus.

In accordance with the method of this invention it is possible to eliminate air agitation of the electrolyte, and all its attending disadvantages, and at the same time to produce electrodeposited sheet metal of notably better uniformity of gage thickness than can be produced with air agitation, by forcibly projecting a turbulent stream of electrolyte into the space between the cathode drum and the adjacent anode, across substantially the entire width of the drum. The stream of electrolyte overflows from the space between cathode and anode without

2

splashing or producing any mist of acid electrolyte droplets. Yet a cathode deposit of remarkable uniformity is produced, which when stripped from the cathode drum forms a sheet of notable uniformity of gage across its width and freedom from objectionable pinholes and other defects.

Preferably the stream of electrolyte is delivered substantially continuously into the space between the cathode drum and the anode, and is introduced into that space 10 adjacent the line of deepest immersion of the cathode drum in the electrolyte. The stream then is projected upwardly in turbulent flow along the surface of each of the two lower quadrants of the drum. Preferably the stream of electrolyte flowing turbulently through the space between cathode drum and anode is maintained substantially free of gas bubbles (especially air or other gas purposely introduced) in order to eliminate to the greatest possible extent the risk of introducing any acid mist into the atmosphere. However, a small amount of 15 air or other gas may be utilized to promote agitation of the electrolyte without sacrificing altogether the improved quality of the electrodeposited sheet that is attained in accordance with the invention.

The apparatus of the invention comprises a cathode 25 drum mounted for rotation on a horizontal axis, a cylindrically curved anode mounted in closely spaced relation with the cathode drum, and means for projecting a turbulent flow of electrolyte into the space between anode and cathode. These means comprise a discharge 30 manifold which extends along an edge of the anode. The discharge manifold comprises an elongated tubular member divided longitudinally into a distribution compartment and a discharge compartment communicating therewith. Means are provided for delivering electrolyte 35 solution into the distribution compartment, and the discharge compartment is provided with a series of spaced solution outlets along substantially the entire length of the discharge manifold. Thus a stream of electrolyte delivered under pressure into said distribution compartment is projected substantially uniformly through said outlets into the space between anode and cathode.

Generally the apparatus comprises a pair of cylindrically curved anodes each mounted in closely spaced relation with one of the lower quadrants of the cathode 45 drum, and with the adjacent edges of the anodes spaced apart substantially along the lowermost portion of the cathode drum. In such apparatus the discharge manifold is preferably positioned between the spaced adjacent edges 50 of the anodes.

A preferred embodiment of the method and apparatus of the invention is described below with reference to the accompanying drawings. While the invention is applicable generally to all metals that can be electrodeposited in sheet form, both the new method and the new apparatus are especially suitable for use in conjunction with the production of sheet copper by electrodeposition from an acidic aqueous copper-bearing electrolyte. Accordingly the following description refers particularly to the 55 production of electrodeposited sheet copper. In the drawings,

Fig. 1 is an elevation, partly in section, through apparatus for producing sheet copper by electrodeposition on a rotating drum cathode;

Fig. 2 is an elevation, partly in section and on an enlarged scale, of the discharge manifold by which electrolyte is projected forcibly into the space between anode and cathode in the apparatus shown in Fig. 1; and

Fig. 3 is a cross section through the discharge manifold taken substantially along the line 3—3 of Fig. 2.

The apparatus shown in Fig. 1 comprises a tank 10 of concrete or other material which is provided interiorly

with a lining 11 of lead and is supported on piers 12. An electrolyte inlet conduit 13 provides for introducing electrolyte intermittently or continuously, as desired, into the tank, and an electrolyte outlet conduit 14 receives the overflow of electrolyte from the tank and provides for maintaining a desired level of electrolyte in the tank. A valved drain pipe 15 is provided for emptying the tank whenever necessary.

A cylindrical cathode drum 16 of lead is supported by an axial shaft 17 which extends through bearings 18 mounted on the sides of the tank 10. The drum is slowly rotated in the direction indicated by the arrows by means of a sprocket chain 19 engaging sprocket wheels 20 and 21 mounted respectively on the drum shaft 17 and on a drive shaft 22. The drive shaft is continuously rotated by a motor (not shown).

The cathode drum 16 extends about half into and half out of the tank 10. A pair of cylindrically curved lead anodes 23 and 24 are mounted in the tank, in close proximity to the two lower quadrants of the cylindrical face of the cathode. Only narrow annular electrolyte spaces 25 and 26 are left between the anodes and the adjacent face of the cathode. The heavy anodes are supported in place by vertical support plates 27 mounted on brick piers 28. Electrical connections to the anodes are made through bus bars 29.

When a direct electric current is passed (at sufficient voltage) from the anodes 23, 24 through copper-bearing electrolyte in the electrolyte spaces 25, 26 to the cathode drum 16, copper is electrodeposited on the cylindrical face of the drum. As the drum rotates, this deposit is carried to above the surface of the electrolyte in the tank 10. There it is separated as a sheet 30 from the face of the drum by passing it over a stripping roll 31, and it is then wound into a coil 32 on a coil core 33. The coil core is mounted on a shaft 34 which is continuously driven by a sprocket chain 35 from the drive shaft 22, in order to maintain the copper sheet 30 under tension as it is stripped from the cathode.

In accordance with the invention, a discharge manifold 36 is mounted between the spaced adjacent lower edges of the anodes 23 and 24, where it extends parallel to the surface of the cathode drum adjacent the line of deepest immersion thereof. The discharge manifold is supported in place by means of a pair of end brackets 37 (only one of which is shown in Fig. 1) and one or more center brackets 38.

The construction of the discharge manifold 36 is shown in detail and on an enlarged scale in Figs. 2 and 3. It comprises lower and upper semi-cylindrical members 39 and 40 (formed, for example, by splitting a lead pipe longitudinally into two equal parts) joined together with a longitudinal partition 41 therebetween and closed at their ends. A solution distribution compartment 42 is defined between the lower member 39 and the partition 41, and a solution discharge compartment 43 is defined between the upper member 40 and the partition 41. The discharge compartment is preferably divided into a plurality of sub-compartments 44 by a series of spaced transverse partitions 45. A solution inlet conduit 46 is provided for admitting electrolyte to the distribution compartment 42. Preferably, as shown, the inlet conduit 46 joins the discharge manifold about at the center thereof; but it can be connected at some other point if design of the apparatus so requires. Each discharge subcompartment 44 is in communication with the distribution compartment 42 through an opening 47 formed in the longitudinal partition 41. These openings 47 are preferably of progressively larger size as they become more remote from the inlet conduit, thereby to insure substantially uniform distribution of solution to each of the discharge sub-compartments 44. At least one and preferably two rows of closely spaced solution outlet openings 48 are formed in the upper member 40 defining the solution discharge compartment. Thus, when solution is delivered to the

discharge manifold through the inlet conduit 46, it is uniformly distributed through the distribution compartment to each discharge subcompartment and therefrom is projected through the discharge openings 48.

As indicated in Fig. 1, the discharge manifold is mounted so that the streams of solution projected from the discharge openings 48 are delivered into the narrow electrolyte spaces 25 and 26 between the anodes and the cathode face of drum 16. The solution inlet conduit 46 is connected to a valved supply pipe 49 through which electrolyte solution under pressure is delivered to the apparatus.

In operation of the above-described apparatus, the tank 10 is filled with a suitable electrolyte, e. g. an acidic aqueous solution of copper sulfate. A source of direct current is connected to the cathode drum 16 and to the anodes 23 and 24. The drive shaft 22 is set in operation, whereby the drum 16 is slowly rotated (in a counter-clockwise direction as viewed in Fig. 1). The voltage between anodes and cathode is high enough so that copper is electrodeposited from the electrolyte in the spaces 25 and 26 between anodes and cathode on to the surface of the cathode drum. As the drum rotates, this electrodeposit is carried to above the surface of the electrolyte in the tank. Conventionally, the deposit on the drum is carefully washed to remove residual electrolyte (by washing means not shown in the drawings). The electrodeposit then is stripped from the face of the drum in the form of the thin sheet 30 and is wound into the coil 32.

The face of the drum from which the copper sheet 30 has been stripped passes under a polishing roll 50 which is continuously rotated at relatively high peripheral speed by a drive chain 51 which connects it to a continuously driven high speed polisher drive shaft 52. The polishing roll 50 maintains a fine smooth surface on the cathode drum to insure the formation of a cathode deposit of good quality and to insure ease of stripping of the deposit from the cathode.

In accordance with the method of the invention, electrolyte solution is introduced continuously and under pressure from the supply pipe 49 through the inlet conduit 46 to the discharge manifold 36. This electrolyte, which enters the distribution compartment 42 and is distributed thereby to the several discharge sub-compartments 44, is forcibly projected as a series of high velocity streams through the discharge outlets 48 into the electrolyte spaces 25 and 26. The electrolyte of these streams, together with electrolyte present in the tank and which is set into circulation by the force of the streams, flows upwardly through the electrolyte spaces toward the surface of the electrolyte at each side of the drum. Thus the electrolyte between the anodes and the cathode is continuously maintained in fast flowing turbulent motion and is continuously renewed and replenished.

The electrodeposited film of copper formed on the cathode drum surface while carrying out the method of this invention is of exceptional uniformity. Its gage thickness across the entire width of the drum is subject to but slight variation, and it is remarkably free of pin-holes and other porosity even when stripped from the drum in sheets of extreme thinness (e. g. one ounce in weight per square foot of surface area, which in the case of copper corresponds to an average gage thickness of only a little over 0.001 inch).

Heretofore it has been common practice to inject air into the electrolyte spaces 25 and 26 between the drum face and the anodes, thereby to promote agitation of the electrolyte adjacent the face of the drum. When employing the method of the present invention, no such air injection is necessary, and in fact it is preferable that the streams of liquid electrolyte projected through the discharge outlets of the manifold 36 be free of any intentionally injected air or other gas. The resulting freedom of the electrolyte from the effects of air agitation results in many improved operating conditions. In particular, the amount of acid electrolyte mist carried into the at-

mosphere is very greatly reduced, with the result that working conditions in the vicinity of the apparatus are greatly improved, the discoloring effect of such mist on the stripped electrodeposited sheet is eliminated, and the corrosive effect of the atmosphere on machine parts is greatly reduced. Also, the splashing and sloshing of electrolyte at its surface level in the tank is eliminated with a number of consequent advantages. Notable among these is the substantial elimination of splashing of the electrolyte on to the surface of the cathode, in the vicinity of the polishing roll 50, which invariably results in occasionally entrapping specks of lead dust generated by the polishing roll 50 and causes them to adhere to the surface of the cathode drum. These specks are then carried on the drum surface to beneath the surface of the electrolyte where they give rise to the defect of "leaded porosity" in the cathode deposit formed on the drum. The elimination of splashing of the electrolyte also greatly reduces the maintenance work required on account of corrosion of machine parts that are necessarily located close to the electrolyte surface.

It is thus apparent that the method and apparatus of this invention make it possible to produce electrodeposited sheet metal of significantly improved quality, and at the same time to greatly improve the operating conditions and to reduce the maintenance work incident to such production.

I claim:

1. Apparatus for producing sheet metal by electro-deposition from an electrolyte solution, comprising a cathode drum mounted for rotation on a horizontal axis, a cylindrically curved anode mounted in closely spaced relation with the cathode drum, and means for projecting a flow of electrolyte into the space between anode and cathode comprising a discharge manifold extending along an edge of the anode, said discharge manifold comprising an elongated tubular member divided longitudinally into a distribution compartment and a discharge compartment communicating with said distribution compartment, means for delivering electrolyte solution into the distribution compartment of said discharge manifold, and said discharge compartment being provided with a series of spaced solution outlets along substantially the entire length of the discharge manifold, said outlets being so positioned as to project a stream of electrolyte delivered under pressure into said distribution compartment into the space between the anode and the cathode drum to cause the electrolyte to flow along the surface of the cathode drum opposite said anode.

2. Apparatus for producing sheet metal by electro-deposition from an electrolyte solution comprising a cathode drum mounted for rotation on a horizontal axis, a pair of cylindrically curved anodes each mounted in closely spaced relation with one of the lower quadrants of the cathode drum, the adjacent edges of said anodes being spaced apart substantially along the lowermost portion of the cathode drum, and means for projecting a flow of electrolyte into the space between anode and cathode comprising a discharge manifold positioned between the spaced adjacent edges of the anodes, said discharge manifold comprising an elongated tubular member divided longitudinally into a distribution compartment and a discharge compartment communicating with said distribution compartment, means for delivering electrolyte solution into the distribution compartment of said discharge manifold, and said discharge compartment being provided with a series of spaced solution outlets along substantially the entire length of the discharge manifold, said outlets being positioned so as to project a stream of electrolyte delivered under pressure into said distribution compartment into the space between the

anode and the cathode drum to cause the electrolyte to flow along the surface of the cathode drum opposite said anode.

3. In apparatus for producing sheet metal by electrodeposition, a discharge manifold comprising an elongated tubular member divided longitudinally into a distribution compartment and a discharge compartment, said compartments being in communication with each other at intervals along the length of the manifold, means for delivering electrolyte solution under pressure into said distribution compartment, and said discharge compartment being formed with a row of closely spaced solution outlets along substantially the entire length of the discharge manifold, whereby a stream of electrolyte solution delivered into the distribution compartment is distributed thereby to the discharge compartment along the length thereof and is projected with substantially uniform force through each of said outlets.

4. In apparatus for producing sheet metal by electrodeposition, a discharge manifold comprising an elongated tubular member divided by a longitudinal partition into a distribution compartment and a discharge compartment, inlet means for introducing electrolyte solution under pressure into said distribution compartment, said partition being formed with a spaced series of openings providing communication between the distribution and discharge compartments, said openings being of progressively larger size as they become more remote from said inlet means, and said discharge compartment being formed with a row of closely spaced solution outlets along substantially the entire length of the discharge manifold, whereby a stream of electrolyte solution delivered into the distribution compartment is distributed thereby to the discharge compartment along the length thereof and is projected with substantially uniform force through each of said outlets.

5. In apparatus for producing sheet metal of electrodeposition, a discharge manifold comprising an elongated tubular member divided by a longitudinal partition into a distribution compartment and a discharge compartment, transverse partitions dividing said discharge compartment into a series of sub-compartments, inlet means for introducing electrolyte solution under pressure into said distribution compartment, said longitudinal partition being formed with a spaced series of openings, each such opening providing communication between one of the sub-compartments of the discharge compartment and the distribution compartment, and such openings becoming progressively larger as they become more remote from said inlet means, and said discharge manifold being formed with a row of discharge openings extending along substantially its entire length, said openings being arranged so that several are provided in each sub-compartment of the discharge compartment, whereby a stream of electrolyte solution delivered into the distribution compartment is distributed thereby substantially uniformly to each sub-compartment and is projected with substantially uniform force through each of said discharge openings.

#### References Cited in the file of this patent

#### UNITED STATES PATENTS

|           |                |                |
|-----------|----------------|----------------|
| 646,313   | Rhodin         | Mar. 27, 1900  |
| 1,760,359 | Hiss           | May 27, 1930   |
| 1,969,054 | Wilkins        | Aug. 7, 1934   |
| 1,991,678 | Jephson        | Feb. 19, 1935  |
| 2,044,415 | Yates          | June 16, 1936  |
| 2,256,729 | Thompson       | Sept. 23, 1941 |
| 2,324,859 | Macan          | July 20, 1943  |
| 2,328,162 | Mercil         | Aug. 31, 1943  |
| 2,477,808 | Jones          | Aug. 2, 1949   |
| 2,569,367 | Bradner et al. | Sept. 25, 1951 |